

## UNITED STATES PATENT OFFICE.

PETER WULFF, OF STARNBERG, AND BRUNO WENDT, OF DESSAU, GERMANY, ASSIGNORS TO I. G. FARBENINDUSTRIE AKTIENGESELLSCHAFT, OF FRANKFORT-ON-THE-MAIN, GERMANY.

## LIGHT-SENSITIVE SILVER HALIDE EMULSIONS AND PROCESS OF MAKING THE SAME.

No Drawing. Application filed May 16, 1927, Serial No. 191,928, and in Germany May 20, 1926.

The present invention relates to light sensitive silver halide emulsions and to a process of making the same. Its object is to obtain valuable light sensitive emulsions from 5 foggy gelatines.

It is known that the ripening process is very important in the manufacture of sensitive silver halide emulsions. The sensitivity attained thereby depends to a great extent on the qualities of the colloid employed, for instance of the gelatin. The ripening capacity of a gelatin may be enhanced by adding substances, the nature and quantity of which depends upon the kind of emulsifying 10 process which is used. These substances are sulphur compounds of a certain constitution, ammonia and others. In this way it is possible to make use of badly ripening gelatin for producing emulsions of the highest sensitivity.

Many sorts of gelatin, however, cannot be used for making sensitive silver halide emulsions because they produce fog before the emulsion has ripened to the sensitiveness desired. Such gelatins have not been applicable hitherto for the production of photographic silver halide emulsion, or they have had to be specially treated before use.

According to the present invention such unsuitable gelatins may be used for making clear emulsions of the highest sensitiveness by adding to the emulsion or to the materials from which it is made, one or more substances which prevent fogging. Appropriate additions for this purpose are certain products of decomposition of proteins which are sometimes incorporated in small quantity in the gelatin, e. g. histidine. Investigation has shown that the tendency towards fogging of many sorts of gelatin in the ripening process is due to the complete or partial lack of these substances which prevent fog. The gelatin may be enriched during its manufacture in its content of the efficacious substances or these latter may be produced separately in order to serve as additions to the colloid before the emulsion is made or to the emulsion in any step of its manufacture or when it is poured on to the support of the emulsion-layer.

Not only the above-mentioned degradation

products of proteins, for example iminazole-alanine, have been found to be suitable additions to emulsions for the purpose in question, but generally iminazole and its derivatives 55 have proved to have an excellent fog preventing action. Their suitability for this purpose is probably due to the fact that the hydrogen-atom of the imino-group can be exchanged for a silver-atom and that adsorption compounds with the silver-salts of the emulsion are formed.

For example, a sensitive silver halide emulsion manufactured according to one of the known processes with a certain sort of 65 gelatin showed considerable fog and little sensitivity. When there is added to the gelatin before or during the making of the emulsion or when the emulsion is poured on the support of the sensitive layer, 0.1-0.4 per 70 cent of nitrobenziminazole a clear and highly sensitive emulsion is obtained.

Having now particularly described and ascertained the nature of our said invention and in what manner the same is to be performed, we declare that what we claim is:

1. Process of manufacturing light-sensitive silver halide emulsions characterized by the step of incorporating in the emulsion a compound of the iminazole-series.

2. Process of manufacturing light-sensitive silver halide emulsions characterized by the step of incorporating in the emulsion a compound of the iminazole-series produced by the degradation of proteins.

3. Process of manufacturing light-sensitive silver halide emulsions characterized by the step of enriching the colloid employed in its content of compounds of the iminazole-series.

4. Light-sensitive silver halide emulsions in which a compound of the iminazole-series is incorporated.

5. Light-sensitive silver halide emulsions in which a compound of the iminazole-series produced by the degradation of proteins is incorporated.

6. Light-sensitive silver halide emulsions in which colloids are incorporated the content of which of compounds of the iminazole-series is enriched.

7. Layers containing light-sensitive silver

halide emulsions in which a compound of the iminazole-series is incorporated.

8. Layers containing light-sensitive silver halide emulsions in which a compound of the iminazole-series produced by the degradation of proteins is incorporated.

9. Layers containing light-sensitive silver

halide emulsions in which colloids are incorporated the content of which of compounds of the iminazole-series is enriched. <sup>10</sup>

In testimony whereof we affix our signatures.

PETER WULFF.  
BRUNO WENDT.